

## UNITED STATES PATENT OFFICE

OLDRICH TUREK, OF PLZEN, CZECHOSLOVAKIA

BLASTING CARTRIDGE, PERCUSSION CAP, DETONATOR, DETONATING FUSE, AND THE  
LIKE

No Drawing. Application filed February 25, 1929, Serial No. 342,672, and in Czechoslovakia March 28, 1928.

2, 4, 6-trinitro 1, 3, 5-triazidobenzene can be suitably employed as priming in detonating caps, if the compression pressure does not exceed 300 kg. cm<sup>2</sup>; otherwise there is a rapid decrease in shattering power and priming force.

The same powerful action which is obtained with the type of detonating caps in which highly compressed 2, 4, 6-trinitro 1, 3, 5-triazidobenzene is combined with highly compressed lead azide, is also obtained with detonating caps, in which use is made, as secondary filling, of highly compressed 2, 4, 6-trinitro 1, 3, 5-triazidobenzene (compression 10 pressure of 300 kg. cm<sup>2</sup> up to 2000 kg. cm<sup>2</sup> and more) and as priming filling a small length of slightly compressed 2, 4, 6-trinitro 1, 3, 5-triazidobenzene. 0.05 grms. to 0.1 grms. of this substance, which has been compressed 15 under a pressure of 300 kg. cm<sup>2</sup> is suitable for the purpose.

As secondary filling in place of highly compressed 2, 4, 6-trinitro 1, 3, 5-triazidobenzene, use can also be made of trinitrotoluene, tetril 25 or other shattering substance; the shattering power of the detonating caps is naturally correspondingly less. 0.5 grms. 2, 4, 6-trinitro 1, 3, 5-triazidobenzene is sufficient for complete priming.

30 What I claim is:—

1. A method of producing blasting cartridges and the like, consisting in filling the detonating cap with compressed 2, 4, 6-trinitro 1, 3, 5-triazidobenzene, serving as secondary filling, and ramming thereupon with a pressure not exceeding 300 kg. cm<sup>2</sup> a priming consisting of 0.05 to 0.2 grms. of 2, 4, 6-trinitro 1, 3, 5-triazidobenzene, as set forth.

2. A method of producing blasting cartridges and the like, consisting in filling the detonating cap with compressed 2, 4, 6-trinitro 1, 3, 5-triazidobenzene, serving as secondary filling, ramming thereupon with a pressure not exceeding 300 kg. cm<sup>2</sup> a priming 40 consisting of 0.05 to 0.02 grms. of 2, 4, 6-trinitro 1, 3, 5-triazidobenzene, and pressing thereon a protective cap with aperture, as set forth.

3. A method of producing blasting cartridges, detonators and the like, consisting in 50

filling a detonating cap with compressed trinitrotoluene, tetryl or other shattering substance (high explosive) serving as secondary filling, ramming thereupon with a pressure not exceeding 300 kg. cm<sup>2</sup> a priming consisting of 0.05 to 0.2 grms. of 2, 4, 6-trinitro 1, 3, 5-triazidobenzene and pressing thereon a protective cap with an aperture, as set forth. 55

In testimony whereof I have signed my name to this specification. 60

OLDRICH TUREK.